

Nov. 23, 1954

A. CASTELLANI  
CONTINUOUS PLASTIC WATERPROOF COATING IN BITUMINOUS GLASS  
ASBESTOS FOR BUILDINGS AND APPLICATION PROCESS THEREOF  
2,695,257  
Filed Dec. 22, 1950



INVENTOR.  
ALDO CASTELLANI

BY  
*Leon M. Straus*  
ACT.

# United States Patent Office

2,695,257

Patented Nov. 23, 1954

1

2,695,257

## CONTINUOUS PLASTIC WATERPROOF COATING IN BITUMINOUS GLASS ASBESTOS FOR BUILDINGS AND APPLICATION PROCESS THEREOF

Aldo Castellani, Livorno, Italy

Application December 22, 1950, Serial No. 202,226

Claims priority, application Italy December 23, 1949

3 Claims. (Cl. 154—128)

This invention relates to a waterproof covering or coating for surfaces, such as roof and like structures, and to a process for preparing the same.

Waterproof coatings or coverings to be useful for roofs must be:

(1) Waterproof under pressures of 3 kilograms per sq. cm. maintained for a one hour period, and under a pressure of 1 kilogram per sq. cm. maintained for an eighteen hour period, in order to provide a factor of safety for conditions normally encountered in use;

(2) Plastic without substantial change in consistency over the range of normal temperatures. To provide for the higher temperature of such coating relative to the surrounding air, the temperature range extends from -10° C. to 50° C. Within this range the coatings should be capable of adjusting to deformation of the underlying structure, whether such deformation is due to the action of heat or displacement of the underlying structure itself.

(3) Stable over prolonged time intervals so that they will not age noticeably, and so that the above-noted properties will be exhibited.

Almost all waterproofing systems are based on the use of hydrocarbons, e. g., asphaltic bitumens, coal tars, native or natural asphalts, and the like, in conjunction with various substances which function as a reinforcing core and simultaneously serve to increase the consistency of the coating. The reinforcing materials usually employed are fibrous fabrics such as paper-wool, hemp, jute, and the like. While reasonably suitable for some purposes, these reinforcing materials for the waterproof coating fail in two fundamental respects, viz., (1) imputrescibility, and (2) ability to leave sufficient plasticity to the coating so that it may follow elastic and thermal deformations of the structure to which it is applied.

The waterproof material should also be stable and insensitive to temperature changes within wide limits.

Heretofore, felted glass fibers have been saturated with petroleum-derived natural asphalt but the coatings or coverings have not proven satisfactory since the asphalt comprised hydrocarbons of various hardness. Furthermore, in forming a coating of several layers it was found that the layers remained separate and distinct rather than bonding together.

It is an object of the present invention to provide an improved waterproof coating or covering for surfaces such as flat roofs, reservoirs, dams, tunnels, freezing plants, and coverings in general.

It is a further object to provide a novel process whereby these improved coatings may be prepared.

These objects are realized by the present invention wherein felted glass fibers are employed as an imputrescible core for the novel waterproof coatings. As the mastic for imparting the waterproof properties there is employed a mixture of asphaltic bitumens or hydrocarbons, about 15-30% of fibrous mineral filler such as asbestos or micro-asbestos, and about 5-15% of finely divided rock asphalt as a filler which improves the weather resistance and stability of the coating or covering (percentages being given by weight). The asphaltic bitumens employed are of high consistency, they are stable both chemically and thermally, and they are devoid of pitch, either vegetal or mineral. Whereas pitch is a synthetic product and comprises the extremely high boiling residue formed in the destructive distillation of wood or coal, for example, the asphaltic bitumens of the present invention are natural, native mixtures of hydrocarbons.

2

More particularly, the asphaltic bitumen comprises a mixture of very hard natural asphalts and petroleum residual asphaltic bitumens as solvent. A preferred composition of the mastic producing superior results comprises about 15-30% of very hard natural asphalts, about 30-50% of petroleum residual asphaltic bitumens as solvent, about 15-30% of fibrous mineral filler, and about 5-15% of finely divided rock asphalt as weather-resistant stabilizing filler.

10 In preparing the novel waterproof coatings or coverings, the base surface is first prepared in conventional manner and a layer of bituminous mastic is applied thereon followed by mopping. A thin layer of felted glass fiber is placed on the mastic and upon the application of heat and pressure the mastic fills the interstices of the glass fiber, serving to embed it within the mastic.

The flow of the mastic may be effected by trailing a warm ironing tool over the felted glass fiber, or by directing a warm jet of compressed air at the surface.

20 These operations may be performed manually or by machines, e. g., a compressed air sprayer of the type employed for road construction and maintenance, blowers, compressors, a battery of jets, and the like. The use of machines will, of course, reduce the amount of time and labor required.

25 It is generally desirable, however, to place the felted glass fibers manually to ensure proper positioning.

The embedding of the felted glass fibers within the mastic may be effected by means of electrically heated mopping tools having a plurality of small spring-loaded 30 pistons. This construction permits substantially uniform application of pressure even where the underlying surface is not perfectly flat.

The invention will be described more fully by reference to the accompanying drawing, in which:

35 Fig. 1 shows a portion of a coating or covering in the preparation stage;

Fig. 2 is a transverse section of a portion of a coating or covering comprising two layers of mastic and felted glass fibers;

40 Fig. 3 is a lateral section of a novel mopping tool; and

Fig. 4 is a bottom plan view of the mopping tool of Fig. 3.

45 In Fig. 1, a layer of mastic 2 is spread on the surface to be protected 1 and a layer of felted glass fibers or glass fiber cloth 3 is disposed on said layer of mastic. The mopping tool 4 operated by handle 5 has been pulled to the right so that the coating on the left side of the figure has been smoothed out while that on the right has not yet 50 been mopped.

55 Fig. 2 shows a coating or covering composed of two such layers of felted glass fibers embedded in mastic. Particularly, a second layer of mastic 2' has been superimposed on said first mopped layer 2. A second layer of felted glass fiber 3' is disposed above layer 2', the fibers of layer 3' extending in transverse direction with respect to the fibers of layer 3. A final layer of mastic 2'' is superimposed on mopped layer 2' and represents the exposed surface. As shown, the several layers of mastic are bonded directly to each other with no discontinuities or air pockets therebetween. Consequently, this preferred covering is composed of (n) layers of bituminous mastic and (n-1) layers of felted glass fibers.

60 The mopping tool of Figs. 3 and 4 comprises a plate 11, electrically heated by passing current through a resistor 19 encased in a housing 12. The housing 12 is fixed in position by nuts which engage threaded vertical rods 17. These vertical rods 17 are connected at their lower ends to plate 11. Adjacent the top of vertical rods 17, upper plate 15 is fastened by nuts. The upper plate 15 is provided with a plurality of holes and plate 11 is also provided with holes, facing those of upper plate 15. Plugs 16 are screwed into the holes in upper plate 15 and pistons 13 extend from each plug 16 and project into the opening in plate 11 so that they contact the base. A compression spring 14 is provided for each piston 13 to maintain the pressure contact between the piston and the base. Eyelets 18 are provided for attaching a handle if desired.

65 In practicing the invention, the first layer of mastic is applied and the reinforcing core, comprising a continu-

## 3

ous felt of glass fibers, is placed thereon with the fibers extending from left to right as shown in Fig. 1.

The plugs 16 of the mop are then actuated to regulate the tension on springs 14. The adjustment is made so that pistons 13 will not protrude beneath the bottom of plate 11. Upon trailing of the tool along the surface of the mastic the mopping is effected by plate 11. If the mastic is not perfectly flat, however, when the plate 11 overlies a depression in the surface, the pistons 13 will be forced downwardly by springs 14. Consequently, pistons 13 will contact the mastic where depressed. As a result the mopping action will be exerted uniformly even where an irregular surface is being worked upon.

After mopping the first layer of mastic, a second layer of mastic is spread out and a second layer of felted glass fibers is superimposed thereon. As shown in Fig. 2, the fibers of the second layer extend in transverse direction with respect to that of the fibers of the first layer. The mopping is repeated and a final layer of mastic is spread out. This layer is also mopped to complete the preparation of the waterproof coating or covering.

As has been indicated, each layer of the reinforcing core comprises a thin layer of felted glass fibers, substantially all of the fibers extending in the same direction. The successive layers of fibers are preferably positioned so that the fibers of any one layer extend in transverse direction with respect to the fibers of adjacent layers. This disposition of the glass fibers produces a far stronger coating which resists sagging, and pulling apart.

While a preferred embodiment of the invention has been shown and herein described, it will be understood that the same is capable of modifications without departure from the general scope and spirit of the invention as defined in the claims.

What I claim is:

1. A waterproof covering for roof and like structures comprising at least two layers of a bituminous mastic, each of said layers having embedded therein a thin stratum of substantially uni-directed felted glass fibers, the fibers of adjacent strata extending in crosswise direction to each other, said bituminous mastic comprising about 15-30% of hard natural asphalt, about 30-50% of petroleum residual asphaltic bitumen as solvent, about 15-30% of fibrous mineral filler, and about 5-15% of finely divided rock asphalt as weather-resistant stabilizing filler, percentages being given by weight.

2. The process for preparing a waterproof covering on a surface, comprising the steps of spreading over the surface to be coated a layer of bituminous mastic comprising about 15-30% of hard natural asphalt, about 30-50% of petroleum residual asphaltic bitumen as solvent, about 15-30% of fibrous mineral filler, and about 5-15% of finely divided rock asphalt as weather-resistant stabilizing

filler percentages being given by weight, placing on said layer a first thin stratum of substantially uni-directed felted glass fibers, applying heat and pressure to said layer and said stratum sufficient to cause said layer to flow between said glass fibers and to embed the same in said layer, spreading a second layer of said mastic over said glass fiber-containing first layer, placing on said second layer a second stratum of uni-directed felted glass fibers, the fibers of said second stratum extending in a transverse direction to the fibers of said first stratum, applying heat and pressure to said second layer and said second stratum to cause said second layer to flow between the glass fibers of said second stratum and to embed said second stratum of glass fibers in said second layer of mastic, and then applying a top coating of mastic to said glass fiber-containing second layer.

3. The process for preparing waterproof coating on a surface, comprising the steps of spreading over the surface to be coated a layer of a bituminous mastic mass having high stability and consistency and a low thermic susceptibility, said bituminous mastic mass being devoid of vegetal and mineral pitch, and comprising about 15-30% of hard natural asphalt, about 30-50% of petroleum asphaltic bitumen as solvent, about 15-30% of fibrous mineral filler, and about 5-15% of finely divided rock asphalt as weather-resistant stabilizing filler, percentages being given by weight, placing on said layer a first stratum of glass fibers all substantially extending in one direction, applying heat and pressure to said layer and said stratum sufficient to cause said layer to flow between said glass fibers and to embed the same in said layer, spreading a second layer of said mastic over said glass fiber-containing first-named layer, placing on said second layer a second stratum of glass fibers extending in a direction different from that of the fibers of said first stratum, applying heat and pressure to said second layer and said second stratum to cause said second layer to flow between the glass fibers of said second stratum and to embed said second stratum of glass fibers in said second layer of mastic, and then applying a top coating of mastic to said glass fiber-containing second layer.

References Cited in the file of this patent

UNITED STATES PATENTS

| Number    | Name           | Date          |
|-----------|----------------|---------------|
| 907,731   | Buckborough    | Dec. 29, 1908 |
| 2,306,347 | Slayer         | Dec. 22, 1942 |
| 2,424,234 | Greider et al. | July 22, 1947 |

OTHER REFERENCES

Miller, "American Roofer," vol. 36, No. 12 (December 1946), pages 12, 13, 25-27 and 29, TH-2431-A1A5.